

## UNITED STATES PATENT OFFICE

2,101,050

## POLISHING COMPOUND

Harry J. Hosking, Sea Cliff, N. Y.

No Drawing. Application December 19, 1936,  
Serial No. 116,821

6 Claims. (Cl. 51—280)

This invention has utility in the art of polishing metallic articles, which involves pressing them upon the surface of a rapidly rotating body which may be a wheel, cylinder, cone, or rapidly moving belt of suitable material.

If the rotating body be a cone, cylinder or wheel, it is usually constructed of disks of cloth of suitable toughness, clamped upon an arbor arranged for rapid rotation, so that the centrifugal force will maintain the disks in extended position, and thus form a fairly rigid surface. The rotating body may also be constructed of bristles, or threads, or cloth, cork or rubber, or wood, the criterion being that the surface shall be soft enough to carry the coating of abrasive herein-after described, and be yielding enough to avoid deformation of the article being polished.

It is customary to coat the rotating surface with an abrasive of suitable hardness and fineness, mixed with grease or with an adhesive or with a mixture of grease and adhesive. This mixture is usually applied in the form of a block, or stick, if it possesses sufficient rigidity to maintain that shape and has a melting point so high that the heat engendered by the friction of the rotating body and the heat of the hand will not soften it so much as to cause it to lose its rigidity.

It may also be encased in paper, or metal or other covering which may be of such consistency as to be worn away along with the abrasive, or it may be scored into narrow strips which may be torn away to expose the abrasive mass.

For special types of finishes there are many objections to the grease-containing abrasive, and also to that which contains both grease and an adhesive. The grease alone has not sufficient adhesive power to resist the centrifugal force and therefore the adhesive does not always form a uniform coating over the surface of the rotating body, but frequently "balls up" thereon.

Also, these grease containing abrasives leave a coating of grease upon the article being polished, which coating must be removed by a subsequent washing with a grease solvent, and drying. Moreover, this film of grease coats the surface so that it is impossible to see the degree of polish which the article has obtained at any given time, until it is removed.

The object of this invention, therefore, is to provide an abrasive compound which is free from the faults above disclosed and free of grease, that is, to produce a greaseless abrasive composition of matter.

This composition must be of sufficient rigidity to maintain its form during use, especially in

warm weather and of a melting point so high that the friction of the rotating body shall not unduly soften it.

Another object of the invention is to provide an abrasive composition that shall spread evenly over the surface of the rotating body, and that shall adhere thereto so that the "balling up" shall not occur.

Another object is an abrasive composition that will leave the polished surface free from any coating derived from the abrasive, and not requiring any subsequent treatment to prepare it for use.

The invention accordingly comprises a composition of matter possessing the characteristics, properties and the relation of constituents which will be exemplified in the composition hereinafter described and the scope of the invention will be indicated in the claims.

My invention is a greaseless abrasive composition of matter, adapted to be pressed against the surface of a rapidly rotating body and to leave upon said surface an even, tightly adherent coating which will not "ball up" nor form chunks, nor be thrown off by centrifugal force, and which will not leave a film upon the articles being polished.

For convenience in the description of the preparation of my composition, I divide the materials entering into it in four parts, as follows:

|           | 30     |
|-----------|--------|
|           | Pounds |
| Water     | 24     |
| Glue X-5A | 22     |
| Glycerine | 2      |
|           | 35     |

|         | 2        |
|---------|----------|
| Shellac | pounds   |
| Borax   | do 1½    |
| Water   | gallon 1 |
|         | 40       |

|            | 1  |
|------------|----|
| Cresophane | 1  |
| Citronella | 1  |
|            | 45 |

|                 | 45     |
|-----------------|--------|
|                 | Pounds |
| Portland cement | 2      |
| Alundum         | 142    |

The following is the process of compounding 50 these materials:

The water of Part one is placed in water-jacketed kettle and the glue, which is preferably finely divided in order to facilitate solution, slowly added with continuous vigorous agitation. 55

When the glue becomes completely dissolved, the glycerine is added and thoroughly mixed in.

In the meantime, the borax of Part two is dissolved in the water, the solution brought to boiling, the shellac gradually added and the boiling continued until it is completely dissolved.

This solution of Part two is then added to the solution of Part one which is still in the jacketed kettle, the water lost from the latter 10 by evaporation restored, the Cresophane and citronella of Part three added, and the whole thoroughly mixed.

The Portland cement of Part four is thoroughly screened to separate any lumps which may be 15 therein, the screening being directly into the mixture in the kettle. This is kept hot and the whole mixture agitated for half an hour.

The mixture is then filled into tubes of convenient size and suitable material, metal tubes 20 being preferred, although paper, cardboard, cellophane may be used.

This composition when pressed upon the rotating body, yields an even coat to its surface, which adheres thereto and does not leave a film upon 25 the surface of the article being polished. The film dries upon the rotating body, and the amount of glycerine used determines the plasticity and hardness of the coat. The amount of glycerine used above is one per cent. For some purposes, 30 especially in polishing large flat work, where flexibility of the glue head is not an important factor, it is preferable to omit the glycerine entirely.

The amount of Portland cement may also be 35 changed, or it may be entirely omitted. Its function is to unite with a portion of the water of the mixture thereby stiffening it, and it also forms a small amount of concrete with the abradant. A variation of its amount will change the hardness 40 of the mass.

The shellac also has the function of hardening and toughening the mixture and its amount can also vary to produce the necessary quality. While the Portland cement adds a certain amount of 45 hardening, the major portion of hardness depends upon the shellac and borax. The Cresophane is a preservative and the citronella is a perfume.

Various changes may be made in this composition. For instance, the alundum may be substituted by any other desired or suitable abrasive. I have used practically all the commercial ones, such as rouge, tripoli, the silicas, and carborundum with good success. In fact, the abrasive 55 chosen should be that one which best works with the particular material being polished.

The shellac may be replaced by other gums and resins, both natural and artificial, and the glycerine by one of the glycols, in whole or in part.

So of the Cresophane and citronella. Any of the well known disinfectants may replace the first, and other odoriferous compounds, the second.

Since certain changes may be made in the above composition of matter and different embodiments of the invention could be made without departing from the scope thereof, it is intended that all matter contained in the above description shall be interpreted as descriptive or illustrative and not in a limiting sense.

It is also to be understood that the following claims are intended to cover all the generic and specific features of the invention described herein and all statements of the scope of the invention which as a matter of language might be said to fall therebetween; and that they are intended to be inclusive in scope and not exclusive, in that, if desired, other materials may be added to my novel composition of matter herein claimed without departing from the spirit of the invention. Particularly it is to be understood that in said claims, ingredients or components recited in the singular are intended to include compatible mixtures of said ingredients wherever the sense permits.

I claim:

1. A composition of matter comprising a mixture of water, glue, glycerine, borax and alundum and the products of their combinations.

2. A composition of matter comprising a mixture of water, glue, glycerine, shellac, borax, Portland cement and alundum.

3. A composition of matter comprising a mixture of glue, shellac, borax, a glue plasticizing material and an abrasive.

4. A composition of matter comprising a mixture of glue, shellac, a shellac softening and dissolving material, a glue plasticizing material and an abrasive.

5. A greaseless polishing compound in the form of a solid mass, comprising glue, a glue plasticizing material, shellac, a shellac dissolving material, an odoriferous compound, a preservative and an abrasive.

6. A composition of matter in the form of a solid mass comprising glue, a glue softening material in amount sufficient to give the composition a suitable degree of hardness, a gum which is soluble in a solution of borax, a disinfectant, an odoriferous material, and an abrasive.

HARRY J. HOSKING. 55